# EUROPEAN PATENT SPECIFICATION

(11) **EP 1 918 393 B1**
(45) Date of publication and mention of the grant of the patent: **22.06.2011**
(21) Application number: 06124232.7
(22) Date of filing: 16.11.2006
(51) Int. Cl.: C22C 21/00, C23F 13/12

(54) **Alloy for use in galvanic protection**
Legierung für Gebrauch im galvanischen Schutz
Alliage pour l'usage dans la protection galvanique

(30) Priority: 03.11.2006 AU 2006235903
(43) Date of publication of application: 07.05.2008
(73) Proprietor: Marine Protection Systems Pty Ltd., Osborne Park, WA 6017 (AU)
(72) Inventor: Maddern, Brett Alexander, Scarborough, Western Australia 6019 (AU)
(74) Representative: Van Breda, Jacobus

(56) References cited:
- JP-A- 2002 097 539
- KR-A- 20050 067 605
- US-A- 3 368 952
- 1 January 1900 (1900-01-01), 19000101 , XP008099770 * abstract * & CHEMICAL ABSTRACTS, vol. 54, no. 2, 1996, Columbus, Ohio, US; abstract no.: 125:336054, OSAMI NAGATA, TAKEUCHI KATSUZI: "Corrosion after 3.5 years' service of an aluminum boat using 6951 alloy brazed honeycomb panels and 6N01-T5 alloy extrusions on her main hull structures" XP008099770
- 19000101, 1 January 1900 (1900-01-01), XP008099771 & CHEMICAL ABSTRACTS, vol. 54, no. 2, 1989, Columbus, Ohio, US; abstract no.: 112:61028, H. MEISSNER: "A review of long-term corrosion tests on aluminum alloys in Arabian Gulf water" page 299 XP008099771

## Description

### FIELD OF THE INVENTION

The present invention relates to an alloy used in the galvanic protection of non metallic water vessels.

### BACKGROUND TO THE INVENTION

In the marine industry the prevention of corrosion of components, such as metal fasteners, shaft and propeller components, constructed from stainless steel and bronze alloys is a primary concern. In aerated marine environments these materials are susceptible to crevice and pitting corrosion. Sacrificial anodes are commonly employed to provide cathodic protection to these components. Application of these sacrificial anodes on wooden and fibreglass vessels can result in an over protection, which may result in a reduced life of coatings and an enhanced level of marine growth and wood rot.

"Corrosion after 3.5 years' service of an aluminium boat", KEIKINZOKU YOSETSU - JOURNAL OF THE LIGHT METAL WELDING ANDCONSTRUCTION, 1996-01-01, authors Nagata O and Takeuchi K, discloses an aluminium alloy composition comprising 0.40-0.9% Si, 0.40-0.8% Mg, 0-0.50% Mn, 0-0.35% Cu, 0-0.35% Fe, 0-0.30% Cr, 0-0.25% Zn, 0-0.1% Ti, balance Al.

The present invention seeks, therefore, among other things, to provide an alloy which overcomes some of the above mentioned disadvantages.

### SUMMARY OF THE INVENTION

An alloy which comprises from 0.30 to 0.6 per cent silicon plus or minus 5 per cent, 0.1 to 0.30 per cent iron plus or minus 5 per cent, 0.10 copper per cent plus or minus 5 per cent, 0.10 per cent manganese plus or minus 5 per cent, 0.35 to 0.6 per cent magnesium plus or minus 5 per cent, 0.05 per cent chromium plus or minus 5 per cent, 0.15 per cent zinc plus or minus 5 per cent, 0.10 per cent titanium plus or minus 5 per cent, 0.05 maximum individual trace metals plus or minus 5 per cent, 0.15 per cent total trace metals plus or minus 5 per cent and the balance aluminium.

### BRIEF DESCRIPTION OF THE DRAWING

In the drawing there is shown Figure 1 which is a schematic side elevation of an anode formed of the alloy of the present invention.

### DESCRIPTION OF THE PREFERRED EMBODIMENTS

In a preferred embodiment of the present invention the metallic components of a water vessel with a non-metallic hull are protected by connecting the alloy of the present invention and the metallic components of the water vessel to form an electrochemical cell. This electrochemical cell is created through the electrical connection of an anode formed of the alloy the present invention to a cathode which are the metallic components of a vessel. The cathode and the anode are both located in a bridging medium. The connection of the anode and the cathode in this way allows for the passage of electrons from the anode to the cathode. These electrons are generated through oxidation of species at the anode and reduction of species at the cathode.

In a galvanic protection system the physical integrity of the anode is sacrificed in order to maintain the physical integrity of the cathode. The physical integrity of the anode is sacrificed through the dissolution of the anode into the bridging medium. The suitability of the anode for galvanic protection is determined by the electrochemical potential of the anode compared to the cathode and the capacity of the anode to protect the cathode.

The alloy forming the anode has a chemical composition comprising 0.30 to 0.6 per cent silicon plus or minus 5 per cent, 0.1 to 0.30 per cent iron plus or minus 5 per cent, 0.10 per cent copper plus or minus 5 per cent, 0.10 per cent manganese plus or minus 5 per cent, 0.35 to 0.6 per cent magnesium plus or minus 5 per cent, 0.05 per cent chromium plus or minus 5 per cent, 0.15 per cent zinc plus or minus 5 per cent, 0.10 per cent titanium plus or minus 5 per cent, 0.05 maximum individual trace metals plus or minus 5 per cent, 0.15 per cent total trace metals plus or minus 5 per cent with the balance being aluminium.

The anode formed of the alloy of the present invention has an electrochemical potential more negative than that of the cathode, preferably with an electrochemical potential in the range of -500 to -1200 mV, more preferably with an electrochemical potential in the range of -500 to -1100 mV,

The capacity of the anode to protect the cathode may be in the range of 1000 to 2000 Ah/kg, preferably in the range of 1400 to 1700 Ah/kg.

The surface area of the anode 10 shown in Figure 1 is increased through the incorporation of ridges 12 on the surface of the anode. The surface area ratio of the anode to the cathode may be in the range of 1:1 to 1:20, preferably in the range of 1:2 to 1:20.

The electrical connection provides a passage for the flow of electrons between the cathode and the anode. The electrical connection is preferably a metallic wire, more preferably a copper wire.

The bridging medium provides a passage for the flow of electrons between the anode and the cathode. The bridging medium is preferably an aqueous solution, more preferably saltwater, particularly sea water.

By applying an excess negative electrochemical potential applied across the cell the accumulation of excess calcium deposits, wood rot and paint disbondment may be prevented. This excess negative electrochemical potential is applied across the cell due to the differences in the electrochemical potential of the anode and the cathode.

In an alternative embodiment of the invention, seawater as a bridging medium may be replaced with another suitable aqueous liquid, preferably brackish water or fresh water.

The anode may be connected to the metallic components of the vessel using known techniques such as connecting the anode to the shaft gland/ seal and, or shaft support bracket and, or the rudder and, or the trimtabs through a bonding buss bar/ system via bonding wire.

The anode of the present invention is particularly envisaged for use with water vessels with fibreglass or wooden hulls,

Modifications or variations as would be apparent to a skilled addressee are deemed to be within the scope of the present invention.

## Claims

1. An alloy which comprises from 0.30 to 0.6 per cent silicon plus or minus 5 per cent, 0.1 to 0.30 per cent iron plus or minus 5 per cent, 0.10 percent copper plus or minus 5 per cent, 0.10 per cent manganese plus or minus 5 per cent, 0.35 to 0.6 per cent magnesium plus or minus 5 per cent, 0.05 per cent chromium plus or minus 5 per cent, 0.15 per cent zinc plus or minus 5 per cent, 0.10 per cent titanium plus or minus 5 per cent, 0.05 maximum individual trace metals plus or minus 5 per cent, 0.15 per cent total trace metals plus or minus 5 per cent and the balance aluminium.

2. An anode formed of an alloy according to claim 1.

3. An anode as according to claim 2, wherein the electrochemical potential of the anode is more negative than that of the cathode.

4. An anode as according to claim 3, wherein the electrochemical potential of the anode is in the range of .500 to -1200 mV.

5. An anode as according to claim 4, wherein the electrochemical potential of the anode is in the range of -500 to -1100 mV,

6. An anode as according to any of the claims 2 to 5, wherein the capacity of the anode to protect the physical integrity of the cathode is in the range of 1000 to 2000 Ah/kg.

7. An anode as according to claim 6, wherein the capacity of the anode to protect the physical integrity of the cathode is in the range of 1400 to 1700 Ah/kg.

8. An anode as according to any of the claims 2 to 7, for use in the galvanic protection of water vessels with non-metallic hulls.

9. An anode as according to claim 8, wherein the vessel is designed for use in seawater.

10. An anode as according to any of the claims 2 to 9, wherein the surface area ratio of the anode to the cathode in the electrochemical cell is in the range of 1:1 to 1:20.

11. An anode as according to claim 10, wherein the surface area ratio of the anode to the cathode is in the range of 1:2 to 1:20.

12. An anode as according to any of the claims 2 to 11, **characterised in that** an excess negative electrochemical potential is applied across the electrochemical cell.

## Patentansprüche

1. Eine Legierung, die aufweist: 0,30% bis 0,6% Silizium plus oder minus 5%, 0,1% bis 0,30% Eisen plus oder minus 5%, 0,10% Kupfer plus oder minus 5%, 0,10% Mangan plus oder minus 5%, 0,35% bis 0,6% Magnesium plus oder minus 5%, 0,05% Chrom plus oder minus 5%, 0,15% Zink plus oder minus 5%, 0,10% Titan plus oder minus 5%, maximal 0,05% einzelne Spurenmetalle plus oder minus 5%, 0,15% Gesamtspurenmetalle plus oder minus 5% und Aluminium als Rest.

2. Eine Anode, die aus einer Legierung gemäß Anspruch 1 gebildet wird.

3. Eine Anode gemäß Anspruch 2, wobei das elektrochemische Potential der Anode negativer als das der Kathode ist.

4. Eine Anode gemäß Anspruch 3, wobei das elektrochemische Potential der Anode im Bereich von -500 mV bis -1200 mV liegt.

5. Eine Anode gemäß Anspruch 4, wobei das elektrochemische Potential der Anode im Bereich von -500 mV bis -1100 mV liegt.

6. Eine Anode gemäß einem der Ansprüche 2 bis 5, wobei die Kapazität der Anode zum Schützen der physikalischen Integrität der Kathode im Bereich von 1000 Ah/kg bis 2000 Ah/kg liegt.

7. Eine Anode gemäß Anspruch 6, wobei die Kapazität der Anode zum Schützen der physikalischen Integrität der Kathode im Bereich von 1400 Ah/kg bis 1700 Ah/kg liegt.

8. Eine Anode gemäß einem der Ansprüche 2 bis 7 zur Verwendung beim galvanischen Schutz von Wasserfahrzeugen mit nicht-metallischem Rumpf.

9. Eine Anode gemäß Anspruch 8, wobei das Wasserfahrzeug zur Nutzung in Meerwasser bestimmt ist.

10. Eine Anode gemäß einem der Ansprüche 2 bis 9, wobei das Oberflächenverhältnis der Anode zu der Kathode in der elektrochemischen Zelle im Bereich von 1:1 bis 1:20 liegt.

11. Eine Anode gemäß Anspruch 10, wobei das Oberflächenverhältnis der Anode zu der Kathode im Bereich von 1:2 bis 1:20 liegt.

12. Eine Anode gemäß einem der Ansprüche 2 bis 11, **dadurch gekennzeichnet, dass** ein überschüssiges negatives elektrochemisches Potential über die elektrochemische Zelle angelegt wird.

## Revendications

1. Alliage composé de 0.30 à 0.6 pour cent de silicium plus ou moins 5 pour cent, 0.1 à 0.30 pour cent de fer plus ou moins 5 pour cent, 0.10 pour cent de cuivre plus ou moins 5 pour cent, 0,10 pour cent de manganèse plus ou moins 5 pour cent, 0.35 à 0.6 pour cent de magnésium plus ou moins 5 pour cent, 0.05 pour cent de chrome plus ou moins 5 pour cent, 0.15 pour cent de zinc plus ou moins 5 pour cent, 0.10 pour cent de titane plus au moins 5 pour cent, 0.05 pour cent au maximum de traces de métaux individuels plus ou moins 5 pour cent, 0.15 pour cent de métaux à l'état de traces au total plus ou moins 5 pour cent, le reste étant de l'aluminium.

2. Anode formée d'un alliage selon la revendication 1.

3. Anode selon la revendication 2, dans laquelle le potentiel électrochimique de l'anode est plus négatif que celui de la cathode.

4. Anode selon la revendication 3, dans lequel le potentiel électrochimique de l'anode est dans l'intervalle de -500 à -1'200 mV.

5. Anode selon la revendication 4, dans laquelle le potentiel électrochimique de l'anode est dans l'intervalle de -500 à -1'100 mV.

6. Anode selon l'une quelconque des revendications 2 à 5, dans laquelle la capacité de l'anode à protéger l'intégrité physique de la cathode est dans l'intervalle de 1'000 à 2'000 Ah/kg.

7. Anode selon la revendication 6, dans laquelle la capacité de l'anode à protéger l'intégrité physique de la cathode est dans l'intervalle de 1'400 à 1'700 Ah/kg.

8. Anode selon l'une quelconque des revendications 2 à 7, destinée à être utilisée dans la protection galvanique de bateaux à coque non métallique oeuvrant dans l'eau.

9. Anode selon la revendication 8, dans laquelle le bateau est destiné à être utilisé dans l'eau de mer.

10. Anode selon l'une quelconque des revendications 2 à 9, dans laquelle le rapport de surface spécifique entre l'anode et la cathode dans la cellule électrochimique est dans l'intervalle de 1:1 à 1:20.

11. Anode selon la revendication 10, dans laquelle le rapport de surface spécifique entre l'anode et la cathode est dans l'intervalle de 1:2 à 1:20.

12. Anode selon l'une quelconque des revendications 2 à 11, **caractérisée en ce qu'**un potentiel électrochimique négatif en excès est appliqué aux bornes de la cellule électrochimique.
